

1

3,342,571  
GASOLINE COMPOSITION CONTAINING  
n-ALKYLTRIMETHYLLEAD

Maurice R. Barusch, Richmond, Wallace L. Richardson, Lafayette, and George J. Kautsky, El Cerrito, Calif., assignors to Chevron Research Company, a corporation of Delaware  
No Drawing. Continuation of application Ser. No. 397,324, Sept. 17, 1964, which is a continuation of application Ser. No. 25,526, Apr. 29, 1960. This application June 9, 1966, Ser. No. 556,523  
2 Claims. (Cl. 44-69)

## ABSTRACT OF THE DISCLOSURE

Hydrocarbon base fuel having a clear Research octane number of at least 95 and from 20 to 60 percent by volume of aromatic hydrocarbons contains from about 0.5 to about 4 milliliters of n-alkyltrimethyllead per gallon, said n-alkyl group containing from 3 to 8 carbon atoms.

This application is a continuation of Maurice R. Barusch, Wallace L. Richardson and George J. Kautsky U. S. application Ser. No. 397,324, filed Sept. 17, 1964, now abandoned, which in turn is a continuation of Maurice R. Barusch, Wallace L. Richardson and George J. Kautsky U. S. application Ser. No. 25,526, filed Apr. 29, 1960, now abandoned.

This invention relates to an improved gasoline composition. More particularly, the invention is concerned with a superior new hydrocarbon fuel of the gasoline boiling range containing n-alkyltrimethyl lead in which the n-alkyl group contains from 3 to 8 carbon atoms.

Gasoline compositions of high octane number are commonly required for modern spark ignition internal combustion automobile and aircraft engines. Engines of these types in general use today are designed with high compression ratios for more efficient operation. Since the present trend is toward engines of still higher compression ratios for increased power and improved performance, there is a constant demand for gasoline compositions of even higher octane number.

Improved methods of refining and blending gasoline base stocks, and additives such as lead tetraethyl, have been employed to meet the demands for higher octane number gasoline compositions. However, it has been generally realized that there is at present a limit to the improvement in octane number that can be obtained by such conventional methods and additives. New gasoline base stocks with the combination of different additives are greatly needed, therefore, to avoid present limitations and provide gasoline compositions of high octane number for future use in automobile and aircraft engines.

It has now been found that a superior new gasoline composition of high octane number is provided by a hydrocarbon base fuel boiling in the gasoline boiling range to which is added n-alkyltrimethyl lead having from 3 to 8 carbon atoms in the alkyl group, in amounts sufficient to improve the octane number, preferably at least 0.5 milliliter per gallon of base fuel.

The improved gasoline compositions of the invention show unexpectedly high octane numbers compared to previously known combinations of hydrocarbon base fuels and additives. Hydrocarbon base fuels, together with the specified n-alkyltrimethyl lead compounds and mixtures thereof in accordance with the invention, have octane numbers which are substantially higher than similar base fuels employing the conventional lead tetraethyl additive in the same lead content. This is surpris-

2

ing since it has been generally accepted heretofore that other lead compounds are distinctly less efficient than lead tetraethyl with respect to octane number improvement.

The hydrocarbon base fuel of the composition, according to the invention, is prepared by conventional refining and blending processes. It normally contains straight-chain paraffins, branched-chain paraffins, olefins, aromatics and naphthenes. Since straight-chain paraffins have a tendency to adversely affect octane number, the content of such hydrocarbons is ordinarily low.

As already mentioned, the base fuel is a hydrocarbon fuel boiling in the gasoline boiling range. Generally described, such fuels have an ASTM (D-86) distillation with an initial boiling point of about 100° F. and a final boiling point of about 425° F. Preferably, the unleaded base fuel has a Research octane number of at least 85 as determined by the accepted CRF engine test method. Also, the base fuel preferably contains at least 20% by volume of aromatic hydrocarbons. Less than 30% by volume of olefinic hydrocarbons are present in the fuel. The total paraffin and naphthene hydrocarbon content of the preferred fuel may be as much as 80% by volume. For best overall engine performance, fuels containing in the range of 20 to 60% by volume of paraffinic and naphthenic hydrocarbons are preferred for volatility and other desirable gasoline characteristics. The more preferred hydrocarbon base fuels are those which contain from 20 to 60% by volume aromatic hydrocarbons and from 0 to 30% by volume of olefinic hydrocarbons. Most preferably, a gasoline having all-around desirable characteristics has a clear octane number of at least 95 and contains about 50 to 60% by volume of paraffin and naphthene hydrocarbons, about 30 to 40% aromatic hydrocarbons and about 5 to 15% olefinic hydrocarbons.

For practical purposes, not more than about 4 milliliters of lead compounds per gallon is ordinarily used in the compositions. If desired, other octane-improving additives may be employed in addition to the n-alkyltrimethyl lead. These include other lead compounds such as lead tetraethyl, carbonyl derivatives of iron and cyclopentadienyl derivatives of metals such as manganese or iron. Other gasoline additives, such as scavengers like ethylene chloride or bromide, oxidation inhibitors, corrosion inhibitors, surface ignition suppressants like phosphorus compounds, detergents, and the like may be present.

The following example illustrates the preparation of n-alkyltrimethyl lead compound in accordance with this invention. Unless otherwise specified the proportions are on a weight basis.

## EXAMPLE

One mole of n-amyl magnesium bromide Grignard reagent in 1 liter of ethyl ether is prepared in the usual manner. To this is added 134 g. (0.465 mole) trimethyl lead chloride and the mixture is stirred and heated under reflux for about 2 hours. The mixture is allowed to stand overnight. It is then added to about 300 ml. of saturated  $\text{NH}_4\text{Cl}$  aqueous solution. The ether layer is separated, water-washed and dried over anhydrous sodium sulfate. The ether is then distilled off and the remaining liquid product is fractionated at 4 mm. Hg pressure. The n-amyltrimethyl lead boils at 63° C. The yield is 73% of theory based on trimethyl lead chloride used.

In further illustration of the superior new gasoline composition of the invention, several compositions and tests thereon are given in the following additional examples. These tests show the improved effect of the combination of the hydrocarbon base fuel with n-alkyltrimethyl lead as compared with fuels containing other lead compounds.

The following table is a summary of the pertinent data of the examples. The type of compositions of the hydrocarbon base fuel is shown with respect to the percent by volume of the paraffins and naphthenes, olefins and aromatics. The clear octane number of the base fuel is also given. This octane number, as already mentioned, is the accepted Research octane number which is usually employed in designating a given gasoline. This method is described as Research Method D-908 in "ASTM Manual of Engine Test Methods for Rating Fuels."

The table shows the effect on octane number by the addition of n-alkyltrimethyl lead containing 3 to 8 carbon atoms in the alkyl group, as compared to lead tetraethyl. The octane number in this comparison is based on the Motor Method D-357 of the "ASTM Manual of Engine Test Methods for Rating Fuels." This method, which is more stringent than the Research Method, illustrates more accurately the desirable qualities of the improved gasoline composition of the invention.

In the table, the effect of n-alkyltrimethyl lead compared with lead tetraethyl, etc., is based on gasoline compositions containing an equal lead concentration. That is to say, that about 3.1 milliliters per gallon of n-amyltrimethyl lead is compared with 3.00 milliliters per gallon lead tetraethyl, while larger amounts of the higher n-alkyl compounds are used because of the difference in densities and molecular weights of the compounds. The "Improvement" is the difference in the octane number

combustion engines, having a clear Research octane number of at least 95, said fuel being characterized in that the hydrocarbon composition contains from 20 to 60% by volume of aromatic hydrocarbons, not more than 5 30% by volume of olefinic hydrocarbons and not more than 60% by volume of paraffinic and naphthenic hydrocarbons, said fuel containing from about 0.5 to about 4 ml. of n-alkyltrimethyllead per gallon, said n-alkyl group containing from 3 to 8 carbon atoms, said fuel having 10 a Motor Method octane number greater than the corresponding octane number of a mixture of said hydrocarbon composition containing a molar equivalent of tetraethyllead.

2. A hydrocarbon base fuel, boiling in the gasoline 15 boiling range, adapted for use in spark ignition internal combustion engines, having a clear Research octane number of at least 95, said fuel being characterized in that the hydrocarbon composition contains from 20 to 60% by volume of aromatic hydrocarbons, not more than 30% by volume of olefinic hydrocarbons and not more than 60% by volume of paraffinic and naphthenic hydrocarbons, said fuel containing from about 0.5 to about 4 ml. of n-amyltrimethyllead per gallon, said fuel having 20 a Motor Method octane number greater than the corresponding octane number of a mixture of said hydrocarbon composition containing a molar equivalent of tetraethyllead.

TABLE

| Ex. No. | n-Alkyl Group | Hydrocarbon Composition                     |                            |                              | Research Octane Unleaded | Motor Octane           |      |      |                 |      |      | Improvement |  |  |
|---------|---------------|---------------------------------------------|----------------------------|------------------------------|--------------------------|------------------------|------|------|-----------------|------|------|-------------|--|--|
|         |               | Paraffins and Naphthenes, Percent by Volume | Olefins, Percent by Volume | Aromatics, Percent by Volume |                          | n-Alkyl Trimethyl Lead |      |      | Tetraethyl Lead |      |      |             |  |  |
|         |               |                                             |                            |                              |                          | ml.                    | gm.  | No.  | ml.             | gm.  | No.  |             |  |  |
| 1.      | Propyl        | 47                                          | 20                         | 33                           | 94.1                     | 2.6                    | 4.52 | 88.5 | 3.0             | 4.94 | 88.3 | 0.2         |  |  |
| 2.      | Butyl         | 47                                          | 20                         | 33                           | 94.1                     | 2.8                    | 4.73 | 88.8 | 3.0             | 4.94 | 88.3 | 0.5         |  |  |
| 3.      | Amyl          | 47                                          | 20                         | 33                           | 94.1                     | 3.1                    | 4.94 | 88.8 | 3.0             | 4.94 | 88.3 | 0.5         |  |  |
| 4.      | Propyl        | 41                                          | 16                         | 43                           | 95.6                     | 2.6                    | 4.52 | 88.2 | 3.0             | 4.94 | 87.8 | 0.4         |  |  |
| 5.      | Butyl         | 41                                          | 16                         | 43                           | 95.6                     | 2.8                    | 4.73 | 88.7 | 3.0             | 4.94 | 87.8 | 0.9         |  |  |
| 6.      | Propyl        | 54                                          | Trace                      | 46                           | 98.1                     | 2.6                    | 4.52 | 96.3 | 3.0             | 4.94 | 95.2 | 1.1         |  |  |
| 7.      | Butyl         | 54                                          | Trace                      | 46                           | 98.1                     | 2.8                    | 4.73 | 96.0 | 3.0             | 4.94 | 95.2 | 0.8         |  |  |
| 8.      | Amyl          | 54                                          | Trace                      | 46                           | 98.1                     | 3.1                    | 4.94 | 95.8 | 3.0             | 4.94 | 95.2 | 0.6         |  |  |

obtained with alkyltrimethyl lead less the octane number obtained with the equivalent amount of lead tetraethyl.

The examples summarized in the above table show that the improved gasoline composition of the invention containing n-alkyltrimethyl lead having 3 to 8 carbon atoms in the n-alkyl group is decidedly better on the basis of octane number rating than comparable gasoline compositions of the type known heretofore. Surprisingly, other alkyl lead compounds give decidedly worse octane numbers than tetraethyl lead. For example, tert.-butyltrimethyl lead in the fuel of Example 4 gives an octane rating of 86.4, 1.4 octane number lower than the 87.8 with tetraethyl lead. Also, n-dodecyltrimethyl lead in the fuel of Example 6 is 85.2, or 2.6 octane numbers worse.

We claim:

1. A hydrocarbon base fuel, boiling in the gasoline boiling range, adapted for use in spark ignition internal

## References Cited

## UNITED STATES PATENTS

|    |           |         |                |       |
|----|-----------|---------|----------------|-------|
| 50 | 1,592,954 | 7/1926  | Midgley        | 44-69 |
|    | 1,949,949 | 3/1934  | Alleman        | 44-69 |
|    | 2,310,376 | 2/1943  | Smyers et al.  | 44-69 |
|    | 2,855,905 | 10/1958 | Hinkamp et al. | 44-69 |
| 55 | 2,862,801 | 12/1958 | De Witt        | 44-69 |

## OTHER REFERENCES

Wagner et al.: "Improved Motor Fuels Through Selective Blending," paper presented before 22nd meeting of the American Petroleum Institute, Nov. 7, 1941, 19 pp.

DANIEL E. WYMAN, Primary Examiner.

Y. H. SMITH, W. J. SHINE, Assistant Examiners.